# EUROPEAN PATENT SPECIFICATION

(11) **EP 0 447 040 B1**
(45) Date of publication and mention of the grant of the patent: **05.06.1996**
(21) Application number: 91301245.6
(22) Date of filing: 15.02.1991
(51) Int. Cl.: B44F 1/06

(54) **Manufacture of simulated lead lights**
Herstellung von simulierten bleigefassten Fenstern
Fabrication d'imitations de vitraux

(30) Priority: 16.02.1990 IE 57890; 22.03.1990 IE 105990
(43) Date of publication of application: 18.09.1991
(73) Proprietor: Coughlan, Thomas Noel, Montenotte, Cork (IE)
(72) Inventor: Coughlan, Thomas Noel, Montenotte, Cork (IE)
(74) Representative: McCarthy, Denis Alexis

(56) References cited:
- EP-A- 0 038 681
- WO-A-86/02599
- GB-A- 2 165 800
- US-A- 4 103 052
- "Introduction to Paint Technology", 4th edition, 1976, pages 74,75.
- "Paint Technology Manuals", 1966, pages 1-3.

## Description

The present invention primarily concerns a method of manufacturing simulated lead lights and stained glass windows of the kind, for example, referred in European Patent Specification No. 0 038 681.

United States Patent Specification No. 4 103 052 discloses a window having the appearance of being a plurality of panes each adjoined to adjacent panes by cross-bars having the triangular cross-section, on each face of the window, which is typical of the cross-bars of wooden divided sash. This appearance is created by printing, of a single design on only one side of the window with only one colour, and incorporating unpainted areas to produce the illusion of three-dimensional depth of a triangular cross-section.

United Kingdom Patent Specification No. GB 2 165 800 discloses a simulated leaded light pattern which is applied to a pane of glass by screen printing onto one face of the glass a pattern of lines of ink, then applying a coarse grit carborundum to the ink so that the carborundum adheres to the ink, curing the ink, then applying a second layer of ink and applying further, fine carborundum to the second layer of ink, curing the material again and then applying a final layer of ink.

The specification of WO 86/02599 discloses a composition for simulated lead strips for leaded windows comprising 50-75 weight % binder, 5-15 weight % pigment, 5-20 weight % oil and 10-30 weight % filling, the binder being a polymer binder, chosen among polyvinyl alcohol based adhesives, polyurethan based adhesives and synthetic rubber based adhesives.

The present invention provides a method of manufacturing a simulated lead light in which simulated opaque lead canes are built up on the surface of a transparent or translucent carrier, comprising the following steps:
(1) applying lines of an opaque paint to the carrier surface, the lines corresponding to the positions of the desired lead canes;
(2) while the paint is still wet, applying transparent or translucent particulate material so that it adheres to the wet paint;
(3) removing surplus unadhered material; and
(4) drying the paint and the adhered particulate material;
By repeating the above steps, the method allows for the build up, in a sandwich-like manner, of one or more layers comprising opaque paint and transparent or translucent particulate material. It is a preferred feature that in applying subsequent layers, a finer grade of particulate material is applied so as to optimally fill any voids in the covering.

Inclusion of transparent or translucent particulate material makes for ease of production of many coloured versions in particular, white, pale grey and pastel colour versions of simulated lead lights.

The method ideally includes a final application of opaque paint prior to final drying and curing.

A number of applications of opaque paint may be employed in order to achieve a desired thickness, the minimum thickness typically being approximately 200 microns (dry film thickness).

In both embodiments, the opaque paint may be based on, for example, two-pack Epoxy resin and preferably includes micaceous iron oxide (MIO) pigment or tinted versions thereof. The preferred MIO epoxy paint gives enhanced durability, opacity and resistance to chemicals and ultra violet radiation.

The opaque paint may include in its composition, at least one metallic pigment and/or other opacifying material such as aluminium, for example, in powdered form, or copper, zinc, stainless steel, lead or chromium. The inclusion of aluminium, for instance, provides a tinting colour. Furthermore, the addition of aluminium in the MIO-containing opaque paint results in enhanced durability.

Therefore, different tinted colour versions of the preferred MIO Epoxy coating may be employed, whilst retaining the aesthetic and durability benefits of the high MIO pigment content of the paint. White or pastel colour versions may also be produced by the method according to the invention.

The opaque paint may be any colour and "Gold leaf" or simulated "Gold leaf", chromium or stainless steel, may optionally be applied over the final layer of opaque paint so as to enhance the decorative effect in addition to providing increased durability.

The above methods may include the use of natural end/or forced drying or curing techniques partially or wholly to dry the paint and particulate material when applied.

The invention will now be described in more detail with reference to the following specific examples:

### Example 1.

(1) An opaque paint, preferably based on micaceous-iron oxide (MIO) pigment dispersed into two-pack epoxy media is applied to the surface of the transparent or translucent carrier by screen printing;
(2) dry transparent or translucent inorganic or organic particulate material, such as for example crushed glass or washed sea sand or powdered plastic of similar particle size (e.g. in the range 120-180 grit size), is applied to, and adheres to, the wet paint;
(3) unadhered particulate material is removed by brushing or compressed air-hose blowing, for example;
(4) the paint and the particulate material adhered thereto are allowed to dry. If desired, the drying process can be speeded up by force drying methods such as stoving, but in that case, only partial curing is effected;
(5) Step (1) above is repeated to overcoat the partially constructed canes, thus providing an overall sandwich effect, the thickness of the overcoat being adjusted as required;
(6) while the paint is still wet, a finer grate (e.g. in the range 320-600 grit size) of particulate material is applied in order to fill voids in the covering applied by step (2) and to enhance the effect and durability of the coating;
(7) step (3) is repeated;
(8) Step (4) is repeated;
(9) Step (5) is repeated:
(10) The canes are then fully dried, preferably using a hard cure method such as staving in order to achieve the desired toughness parameters.

A typical durable simulated lead cane thickness may be built up by the above method to circa 1.5 to 3mm dry film thickness. Accelerated weathering tests showed that full adhesion and coating integrity were retained after testing for over 3000 hours. The test conditions are equivalent to exposure to approximately six years normal weathering.

### EXAMPLE 2.

A typical opaque paint formulation is as follows:
All w/w ratios are given with respect to the weight of the coating.

| | |
|---|---|
| Micaceous iron oxide | 30 - 40% w/w |
| Metallic Powders e.g. leafing aluminium paste. | 2 - 4% w/w |
| Organic or inorganic pigments e.g. Tio₂ or Phthalocyanoblue | 5 - 10% w/w |
| Two-pack epoxy resin | 25 -35% w/w |
| Solvents, for example, glycol ethers higher alcholols or/and aromatic hydrocarbons. | 25 - 30% w/w |
| Additives | 4 - 5% w/w |

The preferred micaceous iron oxide (MIO) epoxy paint may also contain circa 2% to 4% of leafing aluminium paste.

The MIO epoxy paint may be reacted and cured with activators such as polyamide or suitable polyamine types or adducts as desired to suit production curing schedules.

### EXAMPLE 3.

Example of white version of the opaque paint

| | |
|---|---|
| Rutile Titanium dioxide pigment | Circa 30% w/w |
| Two-pack Epoxy Resin | 25 -35% w/w |
| Additives | 4 - 5% w/w |

The formulations given in examples 2 and 3 contain various additives including surfactants, dispersants and rheology control additives such as hydrogenated castor oil, aluminium stearate or Bentonite gellants.

The method allows for various drying or force drying procedures on plastic sheets, for instance, which may not be able to endure high temperatures.

The methods according to the invention allow the use of relatively inexpensive, readily available materials such as the transparent or translucent particulate material.

Though the invention is described above with reference to the manufacture of simulated lead lights, it will be understood that designs other than tradition Tudor type "lead lights" may also be constructed using the method outlined above. Such other designs may be constructed on glass sheets and other plastic sheeting or opaque sheet material such as decorative panels.

## Claims

1. A method of manufacturing a simulated lead light in which simulated opaque lead canes are built up on the surface of a transparent or translucent carrier, comprising the following steps:
(1) applying lines of an opaque paint to the carrier surface, the lines corresponding to the positions of the desired lead canes;
(2) while the paint is still wet, applying transparent or translucent particulate material so that it adheres to wet paint;
(3) removing surplus unadhered material; and
(4) drying the paint and the adhered particulate material.

2. A method according to Claim 1 wherein steps (1) to (4) are subsequently repeated using a finer grade particulate material.

3. A method according to claim 1 or claim 2 including a final application of opaque paint prior to final drying and curing.

4. A method according to any one of the preceding claims wherein the opaque paint is based on two-pack epoxy resin.

5. A method according to any one of the preceding claims wherein the opaque paint includes micaceous-iron oxide pigment or tinted versions thereof.

6. A method according to claim 5 wherein the opaque paint includes in its composition, at least one metallic pigment and/or other opacifying material selected from the following group: aluminium, copper, zinc, stainless steel, lead and chromium.

7. A method according to any one of the preceding claims wherein "gold leaf", simulated "gold leaf", chromium or stainless steel is applied over the final layer of opaque paint.

8. A simulated lead light manufactured according to any one of the preceding claims, comprising a transparent of translucent carrier having lines of opaque paint on its surface, on which lines transparent or translucent particulate material is adhered.

## Patentansprüche

1. Ein Verfahren zur Herstellung eines Bleiglas-Imitats, bei dem lichtundurchlässige Bleibänder (Imitate) auf die Oberfläche eines transparenten bzw. lichtdurchlässigen Trägermaterials aufgebracht werden und das folgende Schritte umfaßt:
(1) Aufbringen lichtundurchlässiger Farblinien auf der Oberfläche des Trägermaterials; die Linien markieren die Lage der Bleibänder.
(2) Aufbringen der transparenten bzw. lichtdurchlässigen Partikel auf die Farbe; die Farbe muß noch feucht sein, damit die Partikel haften bleiben.
(3) Entfernen des überschüssigen losen Materials.
(4) Trocknen der Farbe und der daran haftenden Partikel.

2. Ein Verfahren nach Anforderung 1, bei dem die Schritte (1) bis (4) unter Verwendung feinkörnigerer Partikel wiederholt werden.

3. Ein Verfahren nach Anforderung 1 oder 2, bei dem vor dem abschließenden Trocknen und Härten eine weitere Schicht lichtundurchlässiger Farbe aufgebracht wird.

4. Ein zusätzliches Verfahren nach den vorstehenden Anforderungen, bei dem Zweikomponenten-Epoxidharz als Substrat für die lichtundurchlässige Farbe dient.

5. Ein zusätzliches Verfahren nach den vorstehenden Anforderungen, bei dem die lichtundurchlässige Farbe Eisenglimmer-Pigment oder gefärbte Varianten davon enthält.

6. Ein zusätzliches Verfahren nach Anforderung 5, bei dem die lichtundurchlässige Farbe mindestens ein Metallpigment und/oder anderes Trübungsmaterial aus der folgenden Gruppe enthält: Aluminium, Kupfer, Zink, rostfreier Stahl, Blei und Chrom.

7. Ein zusätzliches Verfahren nach den vorstehenden Anforderungen, bei dem "Blattgold", "Blattgold-Imitat", Chrom oder rostfreier Stahl auf der letzten Schicht lichtundurchlässiger Farbe aufgebracht wird.

8. Ein nach einer der vorstehend beschriebenen Anforderungen hergestelltes Bleiglas-Imitat, bestehend aus einem transparenten bzw. lichtdurchlässigen Trägermaterial, auf dessen Oberfläche Linien aus lichtundurchlässiger Farbe aufgetragen werden, auf der transparente bzw. lichtdurchlässige Partikel angehaftet werden.

## Revendications

1. Méthode de fabrication d'un voyant lumineux conducteur simulé dans lequel des cannes conductrices opaques simulées sont créées sur la surface d'un porteur transparent ou translucide, et comprenant les étapes suivantes :
(1) dos lignes d'une peinture opaque sont appliqués sur la surface du porteur, ces lignes correspondant aux emplacements des cannes conductrices désirées ;
(2) avant que la peinture n'ait séché, une matière particulaire transparente ou translucide est appliquée, adhérant ainsi à la peinture fraîche ;
(3) l'excès de matière n'ayant pas collé est retiré ; et
(4) le peinture et la matière particulaire collée sont séchèes.

2. Méthode similaire à la revendication 1, dans laquelle les étapes (1) à (4) sont ensuite répétées avec utilisation d'une matière particulaire de qualité plus fine.

3. Méthode similaire à la revendication 1, ou à la revendication 2, incluant une dernière application de peinture opaque avant le séchage et le traitement finals.

4. Méthode similaire à l'une quelconque des revendications précédentes, dans laquelle la peinture opaque est à base de résine époxyde binaire.

5. Méthode similaire à l'une quelconque des revendications précédentes, dans laquelle la peinture opaque contient un pigment d'oxyde de fer micacé ou de versions teintées de ce pigment.

6. Méthode similaire à la revendication 5, dans laquelle la composition de la peinture opaque inclut au moins un pigment métallique et/ou d'autres matières opacifiantes appartenant au groupe suivant : aluminium, cuivre, zinc, acier inoxydable, plomb et chrome.

7. Méthode similaire à l'une quelconque des revendications précédentes, dans laquelle de l'"or en feuille", de l'"or en feuille" simulé, due chrome ou de l'acier inoxydable est appliqué sur la dernière couche de peinture opaque.

8. Un voyant lumineux conducteur simulé fabriqué selon l'une quelconque des revendications qui précèdent, comprenant ou porteur transparent ou translucide doté de lignes de peinture opaque sur sa surface, sur lesquelles sont collées des lignes de matière particulaire transparente ou translucide.
